

## UNITED STATES PATENT OFFICE.

EMIL KLEINSCHMIDT, OF FRANKFORT-ON-THE-MAIN, AND CARL FOHR, OF MIESBACH,  
OBERBAYERN, GERMANY.

## MANUFACTURE OF CORES FOR FOUNDRY WORK.

No Drawing.

Application filed August 30, 1921. Serial No. 497,019.

To all whom it may concern:  
Be it known that we, EMIL KLEINSCHMIDT, a citizen of Germany, residing at Hynsperg-street 7, Frankfort-on-the-Main, Germany, 5 and CARL FOHR, a citizen of Germany, residing at Miesbach, Oberbayern, Germany, have invented certain new and useful Improvements in the Manufacture of Cores for Foundry Work (for which we filed applications in Germany, Dec. 18, 1916, and March 10 31, 1919; Austria, May 2, 1919; Hungary, May 22, 1919; Czechoslovakia, July 21, 1919; Switzerland, May 15, 1919; Denmark, June 1919; Sweden, May 24, 1919; Norway, June 15 11, 1919; Netherlands, May 23, 1919), of which the following is a specification.

In making moulds for metal castings there are used as binding agents for the cores preferably such substances as thick 20 oils, viscous vegetable syrup, viscous molasses and the like. All these core binding media have the disadvantage that, owing to their viscosity, they admix with the cores and only with much difficulty, so that a comparatively 25 large quantity of these expensive binding media is necessary.

According to this invention cores for foundry work are produced in such a manner that convenient binding substances 30 atomized by suitable atomizers, e. g. scattering nozzles or wind sifters are incorporated in the core material (sand). As convenient binding agents pitch, asphalt or other bituminous substances and resins are 35 used.

This invention is realized for example in such a manner that pitch is brought by 40 means of scattering nozzles or wind sifters into a finely atomized form or into the form of substantially impalpable powder. Part of this powder, e. g. 2 to 3% is admixed with the core sand as binding agent, whereupon the desired cores are made from the mixture in the usual manner by moulding and drying.

Besides the advantage already mentioned, viz., the considerable economy in expensive binding agents, special advantages are further obtained in so far as the pulverized 50 pitch melts easily in the kiln and consequently produces a great binding effect, imparting considerable resistance to the core. At the casting the fine pitch powder is completely burnt out of the cores where-

by the cores acquire the desired porosity 55 so that the gases can escape easily from the mould.

The pitch which has been finely pulverized in accordance with this invention, does not cake together under normal conditions 60 but remains in the fine amorphous state. It is consequently very handy and it can further be supplied to the foundries directly in the form of fine powder packed in sheet metal drums.

It has been found out further that even considerably smaller quantities of the expensive binding agents, such as pitch, asphalt, resin and the like will be sufficient 70 for the production of cores of sufficient durability if other cheaper binding agents, e. g. inorganic binding agents, dust of brown-coal, peat or lignite or similar substances are added to the pitch, asphalt, resin or the like which have been pulverized 75 according to this invention.

Loam, clay, red clay, kaolin, schistous clay, pozzuolana cement, Portland cement, magnesia cement, lime, gypsum, alkalies, blast furnace dust and the like have proved 80 to be convenient additions.

By the addition of such binding agents the further advantage is obtained that the caking together of the finely pulverized pitch, asphalt or the like when stored is 85 avoided even at higher than normal temperatures.

It is not possible to produce a sufficiently fine powder when pitch, asphalt or the like are disintegrated by means of the usual 90 crushing devices such as crushers or disintegrators. The advantages realized according to the present invention cannot be obtained by the use of such products from disintegration. In order to ensure a good 95 binding of the core mass considerably larger quantities of such products from crushing or disintegration would have to be used.

The mechanical disintegrating processes have further the inconvenience that the disintegration is to be carried through only 100 with difficulty owing to the continuous clogging of the mills, the pulverized product being so sticky that it cannot be stored or transported as the particles would cake up 105 at once.

We claim:—

1. Core material for foundry work con-

taining in intimately mixed condition a binding agent comminuted to a substantially inpalpable powder.

2. Core material for foundry work containing in intimately mixed condition inorganic binding material and an organic binding material reduced to substantially impalpable powder.
3. A core for foundry work containing

distributed therein a binding agent in the <sup>10</sup> form of a substantially impalpable powder.

In testimony whereof we hereunto affix our signatures.

Signed at Frankfort-on-the-Main by—

EMIL KLEINSCHMIDT.

Meisbach, August 5, 1921.

CARL FOHR.